

## UNITED STATES PATENT OFFICE

1,952,137

METHOD OF DRESSING AND TREATING  
FURS

Oscar F. Muller, Glen Ridge, N. J., assignor to  
Nyanza Color & Chemical Co. Inc., New York,  
N. Y., a corporation of New York

No Drawing. Application October 24, 1931,  
Serial No. 570,985

12 Claims. (Cl. 91—68)

This invention relates to improvements in methods for dressing, treating and finishing furs, and has for its particular object the provision of a new method of dressing and treating furs so that the completed furs will be pliable, more waterproof than under present methods of treatment, and will show an enhanced lustre.

Another object of my invention is a method of treating and dressing furs by which their original pliability, lustre and waterproofing qualities, if impaired, may be restored and even improved upon.

Whilst the method of treating and dressing furs herein illustrated is particularly applicable to rabbit and sheepskins, it should be understood that my process is not limited to these particular kind of skins, but is applicable to other and more expensive furs also.

It is well understood that in the treatment of furs at the present time in the processes of washing or mordanting or dyeing to which raw furs are subjected, chemicals are frequently employed having a rather drastic action upon the fur itself, or upon the skin to which the fur is attached. As a result of these washing, mordanting or dyeing processes, many of the natural protective substances resident in the skins or in the fur are removed with a consequent tendency of decreasing the pliability or the lustre or the water resisting qualities of the finished furs contrasted with the natural furs.

In order to overcome some of the defects caused by these washing, cleaning and dyeing operations, it has been heretofore proposed to dress the finished skins with oils and fats of various descriptions so as to restore some of the natural animal fats removed by these operations.

This is especially the case, when, as in the case of cheaper grades of goods, the whole skins together with the hair have been dyed by dipping, instead of by the more subtle brushing process, and the skins, as a consequence, have become hardened.

My improved method of dressing and treating furs is not to subject same to the action of oils or fats which are apt to leave a deposit of oily or greasy matter upon the skins, but I deposit a very fine dry waxy layer on the washed and dyed fur, following this by the usual drumming operations in sawdust or otherwise so that a lustrous dry polish containing a minimum of extraneous wax material will be left upon the fur, which polish will improve the appearance as well as the water resisting qualities of the fur and skin and will also improve the wearing qualities of the fur

while the pliability of the fur is retained or, if impaired by previous dyeing or washing, is restored.

For my improved process, waxes which may be safely used are paraffine, stearine or carnauba wax. These waxes are applied to the fur and skins by being first converted into watery emulsions.

The watery emulsions which I find suitable for use are made with an emulsifying agent such as triethanolamine or ammonium linoleate. As a specific example of a satisfactory waxy emulsion, I use 10 parts of ammonium linoleate to 500 parts of water and to this mixture is added 50 parts of melted carnauba wax.

The liquid used for treating furs is made by adding 4 ounces of the above wax emulsion to a gallon of water and in some cases I prefer to add to the emulsion so employed 2 ounces of a mordant, such as aluminum acetate for each gallon of water used. The complete mixture will therefore consist of 1 gallon of water, 2 ounces of aluminum acetate and 4 ounces of wax emulsion prepared as above described.

The furs are immersed in this luke warm emulsion for approximately 15 to 20 minutes, after which time the superfluous liquid is drained off by centrifuging or otherwise. The furs are then dried, drummed with sawdust and finished in the usual way by which operations a slight protective film of waterproof wax is left upon the surface of the fur and skin.

It should be noted that instead of immersing the furs in this luke warm emulsion, the hair of the furs can be brushed or sprayed with the same liquid above described, the subsequent processes of drying and drumming with sand or sawdust or similar material and finishing being the same as now generally employed.

Instead of the particular waxes named, it is obvious that other waxes may be employed as well as other suitable emulsifying agents without departing from the spirit of my invention.

Having fully described my invention, what I claim is:

1. A method of treating furs by subjecting same to the action of a colloidal wax emulsion, removing the superfluous emulsion and then drying and drumming the fur.

2. The process of treating furs by subjecting same to a luke warm bath of a colloidal wax solution and subsequently drying and drumming the furs.

3. A method of improving the quality of furs by treating the surface of such furs with a col-

70

75

80

85

90

95

100

105

110

oidal wax emulsion and subsequently drying and drumming the furs.

4. A method of improving the quality of furs and skins by subjecting the furs and skins to the action of a colloidal wax emulsion, removing the superfluous emulsion and drying and drumming the furs and skins.

5. A method of treating furs by immersing same in a colloidal emulsion of carnauba wax, removing the excess emulsion and drying and drumming the furs.

6. A method of treating furs by immersing same in a colloidal wax emulsion, removing the superfluous liquid and then drying and drumming the furs.

7. A method of treating furs by applying an aqueous colloidal solution containing a small percentage of wax to the surface of the fur, removing the excess solution from the surface of the fur and then drying and drumming the fur.

8. The process of treating furs by applying a thin layer of emulsified colloidal wax to the surface of said furs, removing the superfluous emul-

sion from said surface and subsequently drying and drumming the furs.

9. The process of treating furs by applying a thin layer of emulsified wax in colloidal state to the surface of said furs.

10. A method of treating furs by subjecting the surface of said furs to the action of a colloidal suspension of carnauba wax in water, removing the superfluous diluent and then drying and drumming the furs.

11. A method of treating dyed furs by applying to their surface an aqueous colloidal suspension of wax to which is added a mordant, comprising an aluminum salt, removing the water by drying and polishing the impregnated furs by drumming.

12. A method of treating dyed furs by applying to their surface a thin aqueous suspension of wax, held in a colloidal state by means of ammonium linoleate, removing the water of the suspension by drying and any loose adhering particles by drumming.

OSCAR F. MULLER.

25

10c

30

10c

35

11c

40

11c

45

12c

50

12c

55

13c

60

13c

65

14c

70

14c

75

15